

## 1

2,982,705

CORROSION PREVENTIVE GALVANIC ANODE  
ZINC ALLOY

Takeshi Sakano, Urawa-shi, Saitama-ken, Akira Masuda, Omiya-shi, Saitama-ken, Kazuo Toda, Urawa-shi, Saitama-ken, and Yoriyasu Atobe, Omiya-shi, Saitama-ken, Japan, assignors to Mitsubishi Kenzoku Kogyo Kabushiki Kaisha, Tokyo-to, Japan

No Drawing. Filed July 15, 1958, Ser. No. 748,601

7 Claims. (Cl. 204—148)

The present invention relates to the prevention of corrosion of ferrous metals, and more particularly to an improved zinc alloy to be used as the anode material for the purpose of preventing corrosion of ship bodies, iron structures or the like.

Heretofore, the galvanic anode serving to protect ship bodies, iron structures or the like from corrosion, generally were metals such as high purity zinc, magnesium, magnesium alloys, aluminum alloys, etc., among which, high purity zinc has been widely employed. The employment of zinc as a galvanic anode has been attempted for many years. However, it has not always been generally used due to the fact that a sufficient corrosion preventive effect could never be attained by the zinc formerly used, because the current-supplying property of zinc is inferior to those of some other metals such as, for example, magnesium or magnesium alloys.

As is well known, the normal electrode potential of pure zinc is —1.01 volt (saturated calomel electrode) which is substantially low as compared with that of iron, namely —0.69 volt. Accordingly, from the theoretical point of view, a sufficient corrosion preventive current can be supplied by use of zinc as an agent for preventing corrosion to iron structures. However, when conventional zinc is used as a galvanic anode in sea water, anode potential rapidly rises with time to such a degree that it fails to function as a protective anode and the reason thereof may be ascribed to the fact that a coating of the corrosion product is massively deposited on the surface of said anode, thereby making said surface highly resistive to the flow of electric current. And it is well known that the greater the amount of impurity contained in the zinc, the greater the above stated tendency becomes.

The study of the deterioration of the zinc as described above resulted in the suggestion of a zinc electrode of high purity. Recently the technique of refining zinc has progressed so remarkably that a zinc product can readily be manufactured the purity of which is as high as 99.995% to 99.999%. Employment of zinc having such high purity can noticeably reduce said deterioration caused by the rising of anode potential by maintaining the anode at a sufficiently low potential for a long period of time, thereby attaining a substantial effectiveness in preventing corrosion. For example, employment of a zinc anode in sea water for 1000 hours resulted in a potential rise of more than —0.8 volt in the case of the zinc of which the purity was 99.6%, but in the case of the zinc the purity of which was 99.99%, anode potential remained at a value of between —1.00 and —0.95 volt, whereby a substantial difference can be recognized between both the above described zinc materials. In accordance with the appreciation of the property of zinc of high purity, use of said pure zinc as the galvanic anode has gradually been practiced. The high purity zinc may

## 2

be regarded as the material for galvanic anodes which is very practical for preventing corrosion to ship bodies, iron structures or the like, because of the cost of said zinc is much lower than that of magnesium or alloys thereof.

As the results of experiments which were carried out for a long period of time in sea water in connection with galvanic anodes made of zinc, the purity of which is from 99.998% to 99.999%, we have found that the high purity zinc which has been considered to be superior material for the galvanic anode can not maintain a sufficient corrosion preventive effect over long periods of time. That is to say, we have observed that even when high purity zinc is used, a corrosion product is deposited on the surface of the metal and the amount of said product increases gradually while it is used, thus causing a gradual rise of anode potential of the zinc, thereby decreasing the effective potential difference which is necessary for generating a protective current and reducing the effect of preventing the corrosion. Furthermore, we have observed by practical tests with ship bodies that the corrosion product covering the anode adheres to the surface so as to form a solid coating and does not readily fall off by contact with sea water during voyage, thus causing insufficient dissolution of the zinc electrode. Therefore, it was found that, even in the case of the high purity which has far better properties as compared with such a low grade zinc as conventional distilled zinc, a sufficient corrosion preventive effect can not always be expected.

Although many attempts were made to overcome the foregoing difficulties and other disadvantages, none, as far as we are aware, was entirely successful when carried into practice commercially on an industrial scale.

It has now been discovered that an alloy can be made having a superior corrosion preventive effect over a long period of time.

It is an object of the present invention to provide an improved zinc alloy for use as a galvanic anode, which is superior to the zinc of high purity from the standpoint of reduction of the corrosion product which is adherently deposited on the anode surface and of maintenance of the same corrosion preventive effect for a longer period of time.

Another object of the invention is to provide a method for treating iron base materials to prevent corrosion.

Other objects and advantages will become apparent from the following description.

Generally speaking, the present invention contemplates a zinc alloy, of the highest purity zinc, and a metal near the center of group III A of the periodic table (in accordance with the Periodic Chart of Elements found on pages 342 and 343 Handbook of Chemistry and Physics, 33rd edition, 1951 and 1952, published by Chemical Rubber Publishing Co., Cleveland, Ohio) (or other editions of the same work). Thus, the useful metals of the group for our purposes can be described as indium and the metals below and on both sides of indium (referring to the above mentioned handbook, as follows:

60

65

|          |          |           |
|----------|----------|-----------|
| 48<br>Cd | 49<br>In | .50<br>Sn |
|          | 81<br>Tl |           |

i.e., elements number 48, 49, 50 and 81, all of them being metals having a low melting point.

These metals having similar properties have a similar effect in improving the property of high purity zinc, so that when two or more of said metals are added together, i.e., used together, equal or multiplied effect will be realized.

The continuous maintenance of such an anode potential, i.e.,  $-1.00 \sim -1.02$  volt, (saturated calomel electrode) as that obtained at the beginning of current supply and the possibility of supplying a sufficient anti-corrosion current which is necessary for protecting the iron structures from corrosion are desirable properties for the galvanic anode to be used in sea water. For obtaining the above-stated properties, it is necessary not only to make the amount of corrosion product being deposited on the surface of the zinc anode small, but also to avoid the rigid adherence of said product to the surface of said anode.

The zinc alloy of this invention is an excellent material for the current-supplying anode, because the corrosion product on the surface of the zinc alloy which is the subject of the present invention will only amount to between  $\frac{1}{3}$  and  $\frac{1}{2}$  of that product in the case of the high purity zinc, even after a long period of time under current supplying conditions. Furthermore, the corrosion product on said zinc alloy is in a soft state similar to that of jelly and can easily be scraped away, the anode potential is always maintained at a value of the order of  $-1.02$  volt, i.e., the anode potential at the initial period of electric current supply, thus causing uniform solubility of the anode metal.

In carrying the invention into practice, it is preferred to use a zinc of the highest purity, above about 99.99% pure and one of the metals of the group of metals near the center of group III A of the periodic table, i.e., elements numbers 48, 49, 50 and 81, or a plurality thereof, in a range of from about 0.01% to about 3%, based on the weight of the zinc.

For the purpose of giving those skilled in the art a better understanding of the invention and a better appreciation of the advantages of the invention, the following illustrative examples are given:

## EXAMPLE I

|                                | Saturated calomel electrode                               |                                          | Corrosion product,<br>Percent |
|--------------------------------|-----------------------------------------------------------|------------------------------------------|-------------------------------|
|                                | Anode potential at the beginning of current supply, volts | Anode potential after 2,000 hours, volts |                               |
| High purity zinc (99.999%)     | $-1.02 \sim -1.03$                                        | $-0.97 \sim -0.89$                       | 11-20                         |
| High purity zinc plus cadmium: |                                                           |                                          |                               |
| Cadmium, percent—              |                                                           |                                          |                               |
| 0.001                          | $-1.02 \sim -1.03$                                        | -0.97                                    | 11                            |
| 0.01                           | $-1.02 \sim -1.03$                                        | -1.01                                    | 5                             |
| 0.1                            | $-1.02 \sim -1.03$                                        | -1.02                                    | 5                             |
| 0.5                            | $-1.02 \sim -1.03$                                        | -1.01                                    | 5                             |
| 1                              | $-1.02 \sim -1.03$                                        | -0.99                                    | 5                             |
| 2                              | $-1.02 \sim -1.03$                                        | -0.97                                    | 6                             |
| 3                              | $-1.02 \sim -1.03$                                        | -0.94                                    | 6                             |

## EXAMPLE II

|                               | Saturated calomel electrode                               |                                          | Corrosion product,<br>Percent |
|-------------------------------|-----------------------------------------------------------|------------------------------------------|-------------------------------|
|                               | Anode potential at the beginning of current supply, volts | Anode potential after 2,000 hours, volts |                               |
| High purity zinc plus indium: |                                                           |                                          |                               |
| Indium, percent—              |                                                           |                                          |                               |
| 0.001                         | $-1.02 \sim -1.03$                                        | -0.97                                    | 13                            |
| 0.01                          | $-1.02 \sim -1.03$                                        | -1.01                                    | 7                             |
| 0.1                           | $-1.02 \sim -1.03$                                        | -1.03                                    | 4                             |
| 0.5                           | $-1.02 \sim -1.03$                                        | -1.02                                    | 4                             |
| 1                             | $-1.02 \sim -1.03$                                        | -1.02                                    | 5                             |
| 2                             | $-1.02 \sim -1.03$                                        | -1.01                                    | 5                             |
| 3                             | $-1.02 \sim -1.03$                                        | -0.98                                    | 6                             |

## EXAMPLE III

|                                    | Saturated calomel electrode                               |                                          | Corrosion product,<br>Percent |
|------------------------------------|-----------------------------------------------------------|------------------------------------------|-------------------------------|
|                                    | Anode potential at the beginning of current supply, volts | Anode potential after 2,000 hours, volts |                               |
| 10 High purity zinc plus thallium: |                                                           |                                          |                               |
| Thallium, percent—                 |                                                           |                                          |                               |
| 0.001                              | -1.00                                                     | -0.97                                    | 12                            |
| 0.01                               | -1.00                                                     | -1.00                                    | 5                             |
| 0.1                                | -1.00                                                     | -1.01                                    | 4                             |
| 1                                  | -1.00                                                     | -1.01                                    | 5                             |
| 2                                  | -1.00                                                     | -0.99                                    | 6                             |
| 2.5                                | -1.00                                                     | -0.95                                    | 8                             |

## EXAMPLE IV

|                            | Saturated calomel electrode                               |                                          | Corrosion product,<br>Percent |
|----------------------------|-----------------------------------------------------------|------------------------------------------|-------------------------------|
|                            | Anode potential at the beginning of current supply, volts | Anode potential after 2,000 hours, volts |                               |
| 20                         |                                                           |                                          |                               |
| 25                         |                                                           |                                          |                               |
| High purity zinc plus tin: |                                                           |                                          |                               |
| Tin, percent—              |                                                           |                                          |                               |
| 0.01                       | $-1.02 \sim -1.03$                                        | -0.97                                    | 11                            |
| 0.05                       | $-1.02 \sim -1.03$                                        | -0.99                                    | 8                             |
| 0.1                        | $-1.02 \sim -1.03$                                        | -1.01                                    | 5                             |
| 0.2                        | $-1.02 \sim -1.03$                                        | -0.99                                    | 7                             |
| 0.5                        | $-1.02 \sim -1.03$                                        | -0.96                                    | 11                            |

## EXAMPLE V

|                                                                   | Saturated calomel electrode                               |                                          | Corrosion product,<br>Percent |
|-------------------------------------------------------------------|-----------------------------------------------------------|------------------------------------------|-------------------------------|
|                                                                   | Anode potential at the beginning of current supply, volts | Anode potential after 2,000 hours, volts |                               |
| 35                                                                |                                                           |                                          |                               |
| 40                                                                |                                                           |                                          |                               |
| High purity zinc plus cadmium plus indium plus thallium plus tin: |                                                           |                                          |                               |
| Cadmium, 0.5%-----                                                |                                                           |                                          |                               |
| Indium, 1.0%-----                                                 | $-1.02 \sim -1.03$                                        | -0.97                                    | 11                            |
| Thallium, 1.0%-----                                               |                                                           |                                          |                               |
| Tin, 0.2%-----                                                    |                                                           |                                          |                               |

<sup>1</sup> Amount of corrosion product adhered to anode  $\times 100$

Amount of dissolved zinc

50 It is to be noted that the present invention is not to be confused with the addition of other metals to zinc, e.g., lead or bismuth. Although when a suitable amount of lead or bismuth is added independently, the property of the pure zinc will be improved somewhat, the improvement so obtained is far below that of the alloy of this invention.

55 Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and claims.

65 We claim:

1. Corrosion preventive galvanic anode consisting of zinc, the purity of which is above about 99.99% pure and at least one element selected from the group consisting of elements numbers 48, 49, 50, 81 in an amount of between about 0.01% and about 3% based on the weight of the zinc.

2. A method of preventing corrosion to iron structures which comprises the steps of using as a galvanic anode, an alloy consisting of zinc the purity of which is above

75

about 99.99% and at least one element selected from the group consisting of indium, thallium, cadmium, tin, and mixtures thereof, in an amount of between about 0.01% and about 3% based on the weight of the zinc.

3. A method as claimed in claim 2, wherein the element selected from the group is indium. 5

4. A method as claimed in claim 2, wherein the element selected from the group is thallium.

5. A method as claimed in claim 2, wherein the element selected from the group is cadmium. 10

6. A method as claimed in claim 2, wherein the element selected from the group is tin.

7. A method as claimed in claim 2, wherein the element

selected from the group is mixtures of indium, thallium, cadmium and tin.

**References Cited in the file of this patent**

**UNITED STATES PATENTS**

Re. 4,048 Lighthall \_\_\_\_\_ June 28, 1870  
2,444,174 Tarr et al. \_\_\_\_\_ June 29, 1948

**FOREIGN PATENTS**

10 15,040 Great Britain \_\_\_\_\_ Dec. 8, 1885

**OTHER REFERENCES**

Metals Handbook, Am. Soc. for Metals, 1948, pages 1077 and 1083.